

# UNITED STATES PATENT OFFICE.

CLEMENT L. PERKINS, OF PITTSBURGH, PENNSYLVANIA, ASSIGNOR TO METALS RECOVERY COMPANY, OF NEW YORK, N. Y., A CORPORATION OF MAINE.

## FLOTATION OF MINERALS.

1,364,306.

Specification of Letters Patent.

Patented Jan. 4, 1921.

No Drawing.

Application filed July 21, 1919. Serial No. 312,249.

*To all whom it may concern:*

Be it known that I, CLEMENT L. PERKINS, a citizen of the United States, residing at Pittsburgh, in the county of Allegheny, 5 State of Pennsylvania, have invented certain new and useful Improvements in Flotation of Minerals; and I do hereby declare the following to be a full, clear, and exact description of the invention, such as will enable others skilled in the art to which it 10 pertains to make and use the same.

This invention relates to the concentration of minerals, such as sulfid ores and the like, by flotation, and is based upon the discovery 15 that improved results can be obtained by carrying out the flotation operation with the addition to the ore or mineral pulp of hydrazins, such as phenyl-hydrazin, etc.

Among the hydrazins and their derivatives, including the hydrazo-compounds or diaryl-hydrazins, which can thus be used, may be mentioned the following:—phenyl-hydrazin, either in the form of the free base or in the form of its salts, such as the hydrochlorid or sulfate; naphthylhydrazin, as the free base or in the form of its salts; para-tolyl-hydrazin; acetic-phenyl-hydrazid,  $\text{CH}_3\text{CO.NH.NH.C}_6\text{H}_5$ ; acetone phenyl-hydrazone  $(\text{CH}_3)_2\text{C}=\text{N.NH.C}_6\text{H}_5$ ; tribrom-30 phenyl-hydrazin; hydrazo-benzene or symmetrical di-phenyl-hydrazin  $\text{C}_6\text{H}_5\text{NH.NH.C}_6\text{H}_5$ ; etc. The hydrazins or their derivatives may be added either in the form of the free base, or in the form of salts thereof 35 with acids. In referring to "hydrazin compounds," therefore, I intend to include the simple and substituted hydrazins and their derivatives, whether in the form of the free base, or in the form of salts thereof.

40 The hydrazin compound which I have found of particular value, and which I therefore recommend, is phenyl-hydrazin ( $\text{C}_6\text{H}_5\text{NH.NH}_2$ ). In using phenyl-hydrazin, it may be incorporated with the ore or 45 mineral pulp in any suitable manner, for example, by introducing it into the tube mill in which the ore is being ground, or by adding it directly in its liquid form to the ore pulp, or by first digesting it with water and 50 adding the resulting product, or by mixing it with an organic liquid mixable therewith.

In general, however, it seems that the hydrazins can be more advantageously added to the pulp immediately before flotation, 55 rather than to the grinding mill. Liquid

compounds, such as phenyl hydrazin, may be added directly; others, *e. g.*, in the form of solutions in water or in various organic solvents.

Phenyl-hydrazin, as well as the other hydrazin compounds, have a marked action as collecting agents; that is, agents which cause a very material increase in the recovery of mineral when used in connection with a suitable frothing agent. The hydrazins themselves nevertheless have a considerable frothing action, and, if used in sufficient amounts, may give good results without the addition of other flotation or frothing agents. The present invention, therefore, includes the improvements in the flotation process in which the hydrazins are themselves used without the addition or admixture of other frothing or flotation agents, as well as the process in which other flotation agents, such as frothing agents, oils, etc., are also used.

After the hydrazin compound, either alone or with other flotation agent or agents, has been thoroughly and uniformly distributed throughout the ore or mineral pulp, 80 the resulting mixture is subjected to a flotation operation, as in an ordinary Calow cell, or in apparatus where the air is incorporated in the ore pulp by mechanical agitation.

It is of advantage in many cases to add to the ore pulp a small amount of alkali, not only when the hydrazin compound is used in the form of a salt, but also when the free base is employed. When a salt of the hydrazin is employed, the alkali may act upon it, to a greater or less extent, to set free the free base, but the action of the alkali appears to be an action upon the ore pulp, or upon the mineral constituents, rather than 95 or in addition to its action upon the salt of the hydrazin used, although I do not desire to limit myself by any theoretical explanation of what the action of the added alkali may be in promoting the flotation operation.

A similar improvement in the process has been noted both when alkali has been used with the free base, and when used with salts of the hydrazin. The alkali may be caustic alkali, such as sodium hydrate, or an 100 alkaline salt, such as sodium carbonate, or even lime or calcium oxid or hydrate can be used. Varying amounts of the alkali can be added, but in many cases it is desirable to add sufficient to give a distinct alkaline reac- 110

tion to the ore pulp during the flotation operation. When sodium hydroxid is used with phenyl-hydrazin it appears possible to use a somewhat reduced amount of phenyl-hydrazin. I have also obtained excellent recoveries when lime was used as the added alkali, even when the lime was added to the ground pulp in the Janney cell, and with the consumption of about from one-fifth to 10 one-fourth pound of phenyl-hydrazin per ton. The lime not only has an alkaline reaction, but it may have a beneficial effect in helping to settle the ore pulp.

The amount of the hydrazin or hydrazin derivatives added may vary somewhat, and 15 may be as little as one-fifth or one-fourth pound per ton of ore; (that is, calculated on the weight of the ore, and not of the ore pulp); but larger amounts may, with 20 advantage, be used, particularly where no added frothing agent or flotation agent is used, and as much as one or one and one-half pounds per ton of ore, or even more, can be used.

25 The hydrazins and hydrazin derivatives have proven to be of particular value in the flotation of copper sulfid ores having a siliceous gangue and containing their floatable or sulfid copper in the form of a mixture of chalcocite and chalcopyrite; that is, so-called porphyry ores, such as those of the Utah Copper Company. When using phenyl and naphthyl hydrazins, the best results 30 appear to be obtained by grinding the ore with water and alkali (NaOH) and then adding the hydrazin to the ground pulp immediately before flotation. The results obtained in this way were better than those 35 obtained by adding the hydrazins in the 40 grinding mill.

Where the phenyl-hydrazin or other hydrazin compound or derivatives is used with other flotation agents, it will materially improve the flotation result by its marked 45 action as a collecting agent. The flotation agent with which the hydrazin compound is added may, therefore, with advantage, be a flotation agent with marked frothing properties, for example, pine oil, or other 50 wood distillation oils, or terpineol, which has marked frothing properties, but practically no collecting properties. When the 55 hydrazin is used with a frothing agent, the valuable collecting properties of the hydrazin will thus be supplemented by the frothing properties of the frothing agent.

60 Where the hydrazin compound is miscible with the other flotation agent or agents with which it is to be used, the agents may be first admixed and compounded to form a composite flotation agent, and the composite agent then added to the ore pulp. When the hydrazin is a solid and not readily soluble or miscible with the ore pulp, it may be 65 ground in the ball mill, or dissolved in a

suitable organic solvent therefor, particularly a solvent which is itself readily miscible with the ore pulp, and the resulting solution then added to the ore pulp. If the hydrazin is soluble in water, it may be added 70 in the form of an aqueous solution.

It is a characteristic of the process of the present invention that the froth obtained is readily broken up, while a relatively clean 75 concentrate and high recovery can, nevertheless, be obtained. The concentrate first obtained, for example, from a rougher cell, can, of course, be further concentrated, and the grade of the concentrate thereby further improved, by treatment in a cleaner 80 cell or cells.

The process of the present invention, in which hydrazins are employed, is somewhat related to the process of my companion application, Serial No. 312,248 filed of even 85 date herewith in which azo-compounds, diazo-compounds, and the like, are employed; but the hydrazins and hydrazin compounds used in the process of the present invention, differ from the azo and diazo 90 compounds by the fact that the two nitrogen atoms, which are characteristic of the hydrazins and hydrazin compounds, are united together by a single bond and likewise have hydrogen united thereto, while the azo and diazo compounds contain the nitrogen atoms joined together by a double bond, and are free from substituted hydrogen atoms.

I claim;

1. The method of effecting the concentration of minerals by flotation, which comprises adding to the mineral pulp a small amount of a hydrazin compound, and subjecting the resulting mixture to a flotation operation; substantially as described. 100

2. The method of effecting the concentration of minerals by flotation, which comprises adding to the mineral pulp a small amount of a hydrazin compound, together with a flotation agent having marked frothing properties, and subjecting the resulting mixture to a flotation operation; substantially as described. 110

3. The method of effecting the concentration of minerals by flotation, which comprises adding to the mineral pulp a small amount of a hydrazin substance, together with sufficient alkali to give to the ore pulp a distinct alkaline reaction; and subjecting the resulting mixture to a flotation operation; substantially as described. 115

4. The method of effecting a concentration of minerals by flotation, which comprises adding to the mineral pulp a small amount of an aryl-hydrazin of the general 125 formula R—NH.NH<sub>2</sub> (where R stands for an aryl radical) and subjecting the resulting mixture to a flotation operation; substantially as described.

5. The method of effecting the concen- 130

tion of minerals by flotation, which comprises adding to the mineral pulp a small amount of phenyl-hydrazin and subjecting the resulting mixture to a flotation operation; substantially as described.

6. The method of effecting the concentration of minerals by flotation, which comprises adding to the mineral pulp a small amount of a hydrazin compound, in the 10 form of a salt thereof with an acid, and subjecting the resulting mixture to a flotation operation.

7. The method of effecting the concentration of minerals by flotation, which comprises adding to the mineral pulp a small 15

amount of phenyl hydrazin, together with sufficient alkali to give to the ore pulp a distinct alkaline reaction, and subjecting the resulting mixture to a flotation operation; substantially as described.

8. The method of effecting the concentration of minerals by flotation, which comprises adding to the mineral pulp a small amount of phenyl hydrazin, together with an agent having good frothing qualities, 25 and subjecting the resulting mixture to a flotation operation; substantially as described.

In testimony whereof I affix my signature.  
CLEMENT L. PERKINS.